

Patented June 26, 1923.

1,460,317

# UNITED STATES PATENT OFFICE.

ANNUAL DUKE, OF MARION, INDIANA.

## COATING COMPOSITION.

No Drawing.

Application filed May 14, 1920. Serial No. 381,448.

*To all whom it may concern:*

Be it known that I, ANNUAL DUKE, a citizen of the United States, residing at Marion, in the county of Grant and State of Indiana, have invented new and useful Improvements in Coating Compositions, of which the following is a specification.

This invention relates to a composition for use upon metal surfaces of all kinds such as steam boilers, pipes, radiators and the like, for preventing leakage of fluid therefrom. The composition will also protect the surfaces coated by it from the action of salt water, prevent rust and a surface treated thereby is very easy to keep clean.

The composition can also be used on automobile tops and the like.

The composition consists of a mixture of lard oil, lubricating oil, white lead, graphite, borax and lamp black, the latter being used to color the composition.

I prefer to use the ingredients in the fol-

lowing proportions, viz: 25 per cent lard oil; 25 per cent lubricating oil, 25 per cent 25 pure white lead, 15 per cent of No. 205 fine graphite, 5 per cent powdered borax and 5 per cent of lamp black.

I prefer to mix the lard oil and lubricating oil with the white lead and then with 30 the other ingredients and thoroughly mix them together or all the ingredients can be mixed together at once.

What I claim is:—

A composition for use upon metallic surfaces for the protection thereof from the elements of erosion consisting of lard oil, lubricating oil and white lead of equal portions mixed with a lesser portion of graphite, and powdered borax and lamp black of 40 equal portions but of less portion than the graphite.

In testimony whereof I affix my signature.

ANNUAL DUKE.